

## UNITED STATES PATENT OFFICE

KARL PRINZ ZU LÖWENSTEIN AND WILHELM MÜLLER, OF BERLIN, GERMANY; OLGA PRINZESSIN ZUR LIPPE, EXECUTRIX OF SAID KARL PRINZ ZU LÖWENSTEIN, DECEASED; ASSIGNEES TO HIRSCH, KUPFER UND MESSINGWERKE AKTIENGESELLSCHAFT, OF FINOW (MARK), GERMANY

## HARD ALLOY

No Drawing. Application filed December 11, 1928, Serial No. 325,404, and in Germany February 11, 1928.

In the last decades a number of alloys of iron with carbon, tungsten and molybdenum distinguished by their unusual hardness and heat stableness has become known. These 5 alloys represent, therefore, an excellent starting material for tools and working implements of all kinds especially drawing stones. But the resistance of these hard metals to chemical influences is comparatively slight, which renders them unsuited for the working of such materials that when being clamped in for being worked affect the tool chemically, especially if the temperature arising during the working procedure 10 has become high by reason of the high working speed. Materials acting in this way are hard rubber, vulcanized fibre, glazed cardboard, pertinax, certain sorts of paper, and similar materials having organic components. To give an example also for an inorganic substance we mention the anhydrous sulphate of calcium ( $\text{CaSO}_4$ ) which, as it seems, impairs the cutting capacity of the drilling and cutting tools by its radical. 15 Now, the present invention relates to an iron alloy which, on the one hand, is, as regards hardness, not inferior to the above-mentioned hard alloys owing to its contents in heavy metals in connection with carbon, and which, on the other hand, represents a 20 chemically nearly unaffected tool substance for the working of materials of the above-stated kinds by reason of an addition of chromium and cobalt, the amount of which depends upon, and stands in a certain relation to, the amount of the heavy metal.

A proportion which is characteristic for the present invention and is, probably the cause of its chemical stableness is this: tungsten:chromium:cobalt=about 8:2:1 (per cent by weight).

Anyhow, the amount of iron should not surpass 55 per cent by weight of the total amount of the alloy. Deviations of the 45 numbers of the proportion stated should, preferably, not exceed 10%.

According to the desired hardness and to the admissible brittleness the proportion of the components tungsten, chromium and cobalt with respect to the amount of the iron,

as well as to the amount of the carbon, (this latter being kept between 1 and 4 per cent) varies. A typical analysis of a tough material of medium hardness is, for instance:

55  
55 per cent of iron,  
32 per cent of tungsten,  
8 per cent of chromium,  
4 per cent of cobalt,  
1 per cent of carbon.

In contradistinction to this composition, 60 a very hard material which is sufficiently tough to be used for the manufacture of cellulose threads is composed as follows:

65  
65 per cent of iron,  
65 per cent of tungsten,  
16 per cent of chromium,  
7 per cent of cobalt,  
2 per cent of carbon.

It is known that in many hard alloys molybdenum can be substituted for the tungsten 70 either totally or to a very large proportion. With alloys according to the present invention such substitution is possible only in a certain measure, viz. at the highest up to 25% of the contents of tungsten; the most favorable percentage in relation to the tungsten is about 12.

For the purpose of increasing the chemical stableness nickel which is, as is known, kindred to cobalt can be substituted for this 80 latter metal up to one half of the amount thereof. But in this respect attention must be paid to the point that in the majority of cases the toughness of the alloy is diminished by said substitution, but its hardness is not 85 increased.

Substituting for the iron another metal which is kindred to it has up to now not proved favorable. This fact is not disproved 90 by the other fact that a small addition of manganese improves the texture of the alloy. Probably manganese acts in this instance merely as a reducing agent.

In order to increase the hardness still more, 95 one or more other known hardening substances, viz. silicium, boron, zirconium, titanium, nitrogen, vanadium, beryllium, cerium, and so on, can be added to the alloy, but the per cent thereof should, at the highest, 100

be 4 per cent, as otherwise the alloy becomes too brittle.

The hard metal alloy described is particularly suitable for the production of projectiles for rifles and other fire-arms, and for the manufacture of projectile casings (shells), also for the points of projectiles of large and small calibers as well as for mines, torpedoes and the like.

10 We claim:

1. A hard alloy having a high mechanical strength and chemical stabilities, suitable for tools and working implements, consisting of from 10 to 33 per cent of iron, 1 to 4 per cent of carbon, 64 to 46 percent of tungsten, 16 to 11.5 per cent of chromium and 8 to 5.5 per cent of cobalt, said three last named substances having among themselves the proportions of 8:2:1, all by weight.

20 2. A hard alloy having a high mechanical strength and chemical stabilities, suitable for tools and working implements, consisting of from 10 to 33 per cent of iron, 1 to 4 per cent of carbon, 48 to 35 per cent of tungsten, 16 to 11 per cent of molybdenum, 16 to 15.5 per cent of chromium and 8 to 5.5 per cent of cobalt, the ratio of the total percentage of tungsten and molybdenum to that of chromium and that of cobalt being 8:2:1.

30 3. A hard alloy having a high mechanical strength and chemical stabilities, suitable for tools and working implements consisting of from 10 to 33 per cent of iron, 1 to 4 per cent of carbon, 64 to 46 per cent of tungsten, 16 to 11.5 per cent of chromium, 4 to 3 per cent of cobalt and 4 to 3 per cent of nickel, the ratio of the total percentage of tungsten to that of chromium and that of cobalt and nickel being 8:2:1.

40 4. A hard alloy having a high mechanical strength and chemical stabilities, suitable for tools and working implements consisting of 10 to 33 per cent of iron, 1 to 4 per cent of carbon, 48 to 35 per cent of tungsten, 16 to 11 per cent of molybdenum, 16 to 5.5 per cent of chromium, 4 to 3 per cent of cobalt and 4 to 3 per cent of nickel, the ratio of the total percentage of tungsten and molybdenum to that of chromium and to that of cobalt and nickel being 8:2:1.

In testimony whereof we affix our signatures.

KARL PRINZ ZU LÖWENSTEIN.

WILHELM MÜLLER.